# EUROPEAN PATENT SPECIFICATION

(11) **EP 3 184 661 B1**
(45) Date of publication and mention of the grant of the patent: **22.04.2020**
(21) Application number: 15833925.9
(22) Date of filing: 24.06.2015
(51) Int. Cl.: C22C 38/00, C22C 38/02, C22C 38/06, C22C 38/04, C22C 38/60, C22C 38/34, C22C 38/08, C22C 38/16, C22C 38/10, C21D 8/12, H01F 1/16, H01F 1/147

(54) **NON-ORIENTED ELECTRICAL STEEL SHEET HAVING EXCELLENT MAGNETIC PROPERTIES**
UNGERICHTETES ELEKTROBLECH MIT HERVORRAGENDEN MAGNETISCHEN EIGENSCHAFTEN
TÔLE D'ACIER ÉLÉCTRIQUE NON ORIENTÉE PRÉSENTANT DES PROPRIÉTÉS MAGNÉTIQUES EXCELLENTES

(30) Priority: 20.08.2014 JP 2014167609
(43) Date of publication of application: 28.06.2017
(73) Proprietor: JFE Steel Corporation, Tokyo 100-0011 (JP)
(72) Inventor: NAKAJIMA Hiroaki, Tokyo 100-0011 (JP); OKUBO Tomoyuki, Tokyo 100-0011 (JP); NAKANISHI Tadashi, Tokyo 100-0011 (JP); ODA Yoshihiko, Tokyo 100-0011 (JP)
(74) Representative: Haseltine Lake Kempner LLP
(86) International application number: PCT/JP2015/068123
(87) International publication number: WO 2016/027565

(56) References cited:
- EP-A1- 1 791 985
- EP-A1- 2 657 355
- WO-A1-2013/137092
- WO-A1-2014/027452
- JP-A- H03 219 020
- JP-A- H08 157 966
- JP-A- H08 157 966
- JP-A- 2000 273 549
- JP-A- 2000 328 207
- JP-A- 2000 328 207
- JP-A- 2001 158 949
- JP-A- 2007 031 793
- JP-A- 2012 001 772

## Description

### TECHNICAL FIELD

This invention relates to a non-oriented electrical steel sheet, and concretely to a non-oriented electrical steel sheet having excellent magnetic properties.

### RELATED ART

A non-oriented electrical steel sheet is a type of soft magnetic material widely used as an iron core material for rotors and the like. In the recent trend of energy saving, there are increasing demands for efficiency improvement, downsizing and weight reduction of electrical machineries, and hence it becomes more important to improve magnetic properties of the iron core material.

The non-electrical steel sheet is usually produced by subjecting a raw steel material (slab) containing silicon to hot rolling, hot-band annealing if necessary, cold rolling and finish annealing. In order to realize excellent magnetic properties, it is required to obtain a texture suitable for the magnetic properties at a stage after the finish annealing. To this end, the hot-band annealing is considered to be essential.

However, the addition of the hot band annealing process has a problem that not only the number of days for production becomes long but also the production cost is increased. In particular, an increase of the productivity and a decrease of the production cost recently start to be considered important in association with an increase of demands for the electrical steel sheet, and hence techniques of omitting the hot band annealing have been actively developed.

As the technique of omitting the hot-band annealing, for example, Patent Document 1 discloses a method of improving magnetic properties by decreasing S content to not more than 0.0015 mass% to improve growth of crystal grains, adding Sb and Sn to suppress nitriding of the surface layer, and winding the sheet at a high temperature during the hot rolling to coarsen the crystal grain size of the hot rolled sheet having an influence on the magnetic flux density.

Patent Document 2 discloses a technique as to a production method of a non-oriented electrical steel sheet wherein an iron loss is decreased and a magnetic flux density is increased without conducting the hot band annealing by controlling alloy-component elements, optimizing hot rolling conditions and using phase transformation of steel to control hot-rolled texture.

WO 2013/137092 A1 discloses a method for producing a non-oriented electrical steel sheet having excellent magnetic properties of high magnetic flux density and low core loss.

### PRIOR ART DOCUMENTS

### PATENT DOCUMENTS

Patent Document 1: JP-A-2000-273549
Patent Document 2: JP-A-2008-524449

### SUMMARY OF THE INVENTION

### TASK TO BE SOLVED BY THE INVENTION

In the method disclosed in Patent Document 1, however, it is necessary to reduce S content to an extremely low amount, so that the production cost (desulfurization cost) is increased. Also, in the method of Patent Document 2, there are many restrictions on steel ingredients and hot rolling conditions, so that there is a problem that the actual production is difficult.

The invention is made in view of the above problems of the conventional art, and an object thereof is to provide a non-oriented electrical steel sheet having excellent magnetic properties at a low cost even if the hot band annealing is omitted.

### SOLUTION FOR TASK

The inventors have focused on an influence of impurities inevitably contained in the raw steel material upon the magnetic properties and made various studies for solving the above task. As a result, it has been found out that the magnetic flux density and the iron loss property can be significantly increased by particularly decreasing Ga among the inevitable impurities to an extremely low amount or further decreasing A1 to an extremely low amount even if the hot band annealing is omitted, and the invention has been accomplished.

The invention is defined in the claims.

### EFFECT OF THE INVENTION

According to the invention, the non-oriented electrical steel sheet having excellent magnetic properties can be produced even if the hot band annealing is omitted, so that it is possible to provide non-oriented electrical steel sheets having excellent magnetic properties at a low cost in a short period of time.

### BRIEF DESCRIPTION OF THE DRAWINGS

FIG. 1 is a graph showing an influence of Ga content upon a magnetic flux density B₅₀.
FIG. 2 is a graph showing an influence of A1 content upon a magnetic flux density B₅₀.

### EMBODIMENTS FOR CARRYING OUT THE INVENTION

First, experiments building a momentum on the development of the invention will be described.

### <Experiment 1>

The inventors have investigated an influence of Ga content as an inevitable impurity upon the magnetic flux density in order to develop a non-oriented electrical steel sheet having excellent magnetic properties even if the hot-band annealing is omitted.

Steels prepared by variously changing an addition amount of Ga within a range of tr.-0.002 mass% in a chemical composition system comprising C: 0.0025 mass%, Si: 3.0 mass%, Mn: 0.25 mass%, P: 0.01 mass%, N: 0.002 mass%, S: 0.002 mass% and Al: two levels of 0.2 mass% and 0.002 mass% are melted and casted in a laboratorial way to form steel ingots, which are hot rolled to form hot rolled sheets of 3.0 mm in thickness and subjected to a heat treatment corresponding to a coiling temperature of 750°C. Thereafter, the hot rolled sheets are pickled without conducting a hot band annealing and cold rolled to form cold rolled sheets having a thickness of 0.50 mm, which are subjected to a finish annealing at 1000°C for 10 seconds under an atmosphere of 20 vol% H₂ - 80 vol% N₂.

Magnetic flux densities B₅₀ of the thus obtained steel sheets after the finish annealing are measured by a 25 cm Epstein method to obtain results shown in FIG. 1.

As seen from the results, the magnetic flux density B₅₀ is rapidly increased when the Ga content is not more than 0.0005 mass%, and the effect of increasing the magnetic flux density due to the decrease of Ga content is larger when Al content is 0.002 mass% than 0.2 mass%.

### <Experiment 2>

The inventors have conducted an experiment for investigating an influence of Al content upon the magnetic flux density.

Steels prepared by variously changing an addition amount of Al within a range of tr.-0.01 mass% in a chemical composition system comprising C: 0.0025 mass%, Si: 3.0 mass%, Mn: 0.25 mass%, P: 0.01 mass%, N: 0.002 mass%, S: 0.002 mass% and Ga decreased to 0.0002 mass % are melted in a laboratorial way and magnetic flux densities B₅₀ of the steel sheets after the finish annealing in the same way as in Experiment 1 are measured by a 25 cm Epstein method.

FIG. 2 shows a relation between Al content and magnetic flux density B₅₀ with respect to the above measured results. As seen from this figure, the magnetic flux density is increased when Al content is not more than 0.005 mass%.

As seen from the above experimental results, the magnetic flux density can be significantly increased by decreasing Ga content to not more than 0.0005 mass% or further by decreasing Ga content to not more than 0.0005 mass% while decreasing Al content to not more than 0.005 mass%.

The reason why the magnetic flux density is significantly increased by the decreases of Ga content and Al content is not sufficiently clear yet, but it is presumed that the recrystallization temperature of the raw material is lowered by decreasing Ga to change recrystallization behavior in the hot rolling to thereby improve the texture of the hot rolled sheet. Particularly, the reason why the magnetic flux density is considerably increased when Al content is not more than 0.005 mass% is considered due to the fact that mobility of grain boundary is changed by the decrease of Ga and Al to promote growth of crystal orientation advantageous for the magnetic properties.

The invention is developed based on the above new knowledge.

Next, there will be explained a chemical composition required in the non-oriented electrical steel sheet according to the invention.

### C: not more than 0.01 mass%

C causes magnetic aging in a product sheet, so that it is limited to not more than 0.01 mass%. Preferably, it is not more than 0.005 mass%.

### Si: not more than 6 mass%

Si is an element effective of increasing a specific resistance of steel to decrease an iron loss, so that it is preferable to be contained in an amount of not less than 1 mass%. When it is added in an amount exceeding 6 mass%, however, it is difficult to perform cold rolling because considerable embrittlement is caused, so that the upper limit is set to 6 mass%. Preferably, it is a range of 1-4 mass%, and more preferably a range of 1.5-3 mass%.

### Mn: 0.05-3 mass%

Mn is an element effective for preventing red brittleness in the hot rolling, and therefore it is required to be contained in an amount of not less than 0.05 mass%. When it exceeds 3 mass%, however, cold rolling property is deteriorated or decrease of the magnetic flux density is caused, so that the upper limit is set to 3 mass%. Preferably, it is a range of 0.05-1.5 mass%. More preferably, it is a range of 0.2-1.3 mass%.

### P: not more than 0.2 mass%

P can be added because it is excellent in the solid-solution strengthening ability and is an element effective of adjusting hardness to improve punchability of steel. However, when the amount exceeds 0.2 mass%, embrittlement becomes remarkable, so that the upper limit is set to 0.2 mass%. Preferably, it is not more than 0.15 mass%, more preferably not more than 0.1 mass%.

### S: not more than 0.01 mass%

S is a harmful element forming sulfide such as MnS or the like to increase the iron loss, so that the upper limit is set to 0.01 mass%. Preferably, it is not more than 0.005 mass%, and more preferably not more than 0.003 mass%.

### Al: not more than 2 mass%

Al can be added because it is an element effective of increasing a specific resistance of steel to decrease an eddy current loss. However, when it exceeds 2.0 mass%, the cold rolling property is deteriorated, so that the upper limit is set to 2.0 mass%.

In order to more receive the effect of improving the magnetic properties by the decrease of Ga, it is preferable to be decreased to not more than 0.005 mass%. More preferably, it is not more than 0.001 mass%.

### N: not more than 0.005 mass%

N is a harmful element forming nitride to increase the iron loss, so that the upper limit is set to 0.005 mass%. Preferably, it is not more than 0.003 mass%.

### Ga: not more than 0.0005 mass%

Ga is the most important element in the invention because it has a substantial bad influence on a texture of a hot rolled sheet even in a slight amount. In order to suppress the bad influence, it is necessary to be not more than 0.0005 mass%. Preferbly, it is not more than 0.0001 mass%.

The non-oriented electrical steel sheet according to the invention may contain one or two of Sn and Sb in ranges of Sb: 0.01-0.2 mass% and Sn: 0.01-0.2 mass% in addition to the above ingredients for improving the magnetic properties.

Sb and Sn improve a texture of a product sheet and are elements effective for increasing the magnetic flux density. The above effect is obtained in an addition amount of not less than 0.01 mass%. On the other hand, when it exceeds 0.2 mass%, the above effect is saturated. Therefore, in the case of adding the elements, the each element is in a range of 0.01-0.2 mass%. More preferably, it is a range of Sb: 0.02-0.15 mass% and Sn: 0.02-0.15 mass%.

The non-oriented electrical steel sheet according to the invention may further contain one or more selected from Ca, REM and Mg in ranges of Ca: 0.0005-0.03 mass%, REM: 0.0005-0.03 mass% and Mg: 0.0005-0.03 mass% in addition to the above ingredients.

Each of Ca, REM and Mg fixes S to suppress fine precipitation of sulfide and is an element effective for decreasing the iron loss. In order to obtain such an effect, the each element is required to be added in an amount of not less than 0.0005 mass%. However, when it is added in an amount exceeding 0.03 mass%, the effect is saturated. Therefore, in the case of adding Ca, REM and Mg, the each element is in a range of 0.0005-0.03 mass%. More preferably, it is a range of 0.001-0.01 mass%.

The non-oriented electrical steel sheet according to the invention may further contain one or more selected from Ni, Co, Cu and Cr in ranges of Ni: 0.01-2.0 mass%, Co: 0.01-2.0 mass%, Cu: 0.03-5.0 mass% and Cr: 0.05-5.0 mass% in addition to the above ingredients.

Ni, Co, Cu and Cr are elements effective for decreasing the iron loss because the each element increases the specific resistance of steel. In order to obtain such an effect, it is preferable to add Ni and Co in an amount of not less than 0.01 mass% for each, Cu in an amount of not less than 0.03 mass% and Cr in an amount of not less than 0.05 mass%. However, when Ni and Co are added in an amount exceeding 2.0 mass% and Cu and Cr are added in an amount exceeding 5.0 mass%, an alloy cost is increased. Therefore, in the case of adding Ni and Co, the each amount is a range of 0.01-2.0 mass%, and in the case of adding Cu, the amount is a range of 0.03-5.0 mass%, and in the case of adding Cr, the amount is a range of 0.05-5.0 mass%. More preferably, it is Ni: 0.03-1.5 mass%, Co: 0.03-1.5 mass%, Cu: 0.05-3.0 mass% and Cr: 0.1-3.0 mass%.

The remainder other than the above ingredients in the non-oriented electrical steel sheet according to the invention is Fe and inevitable impurities. However, the addition of other elements may be accepted within a range not damaging the effects of the invention.

Next, the method of producing the non-oriented electrical steel sheet according to the invention will be described below.

The non-oriented electrical steel sheet according to the invention can be produced by the conventionally well-known production method for the non-oriented electrical steel sheet as long as Ga and Al are contained in the aforementioned ranges as a raw material used in the production. For example, it can be produced by a method wherein a steel adjusted to have the predetermined chemical composition in a refining process of melting the steel in a converter, an electric furnace or the like and performing secondary refining in a vacuum degassing apparatus or the like is subjected to an ingot making-blooming method or continuous casting to form a raw steel material (slab), which is then subjected to hot rolling, pickling, cold rolling, finish annealing, and an application and baking of an insulation coating.

In the production method of the non-oriented electrical steel sheet according to the invention, excellent magnetic properties can be obtained even if the hot band annealing after the hot rolling is omitted. However, the hot band annealing may be conducted, and at this time, a soaking temperature is preferable to be a range of 900-1200°C. When the soaking temperature is lower than 900°C, the effect by the hot band annealing cannot be obtained sufficiently and hence the effect of further improving the magnetic properties cannot be obtained. On the other hand, when it exceeds 1200°C, the grain size of the hot rolled sheet is coarsened too much, and there is a fear of causing cracks or fractures during the cold rolling and it becomes disadvantageous to the cost.

Also, the cold rolling rolling from the hot rolled sheet to the cold rolled sheet with a product sheet thickness (final thickness) may be conducted once or twice or more interposing an intermediate annealing therebetween. In particular, the final cold rolling to the final thickness is preferable to be a warm rolling performed at a sheet temperature raised to approximately 200°C because it has a large effect of increasing the magnetic flux density as long as there is no problem in equipment, production constraint or cost.

The finish annealing subjected to the cold rolled sheet with the final thickness is preferable to be a continuous annealing performed by soaking at a temperature of 900-1150°C for 5-60 seconds. When the soaking temperature is lower than 900°C, the recrystallization is not promoted sufficiently and good magnetic properties are not obtained. While when it exceeds 1150°C, crystal grains are coarsened and the iron loss at a high frequency zone is particularly increased.

The steel sheet after the finish annealing is preferable to be coated on its surface with an insulation coating for increasing interlayer resistance to decrease the iron loss. It is particularly desirable to apply a semi-organic insulation coating containing a resin for ensuring a good punchability.

The non-oriented electrical steel sheet coated with the insulation coating may be used after subjected to a stress relief annealing by users, or may be used without the stress relief annealing. Also, a stress relief annealing may be performed after a punching process is conducted by users. The stress relief annealing is usually performed under a condition of about 750°C for 2 hours.

### EXAMPLE

Steels No. 1-31 having a chemical composition shown in Table 1 are melted in a refining process of convertor-vacuum degassing treatment and continuously casted to form steel slabs, which are heated at a temperature of 1140°C for 1 hour and hot rolled at a finish hot rolling temperature of 900°C to form hot rolled sheets having a sheet thickness of 3.0 mm, and wound around a coil at a temperature of 750°C. Next, the coil is pickled without being subjected to a hot band annealing, and cold rolled once to provide a cold rolled sheet having a sheet thickness of 0.5 mm, which is subjected to a finish annealing under soaking conditions of 1000°C and 10 seconds to provide a non-oriented electrical steel sheet.

From the thus obtained steel sheet are taken out Epstein test specimens with 30 mm ×280 mm to measure an iron loss W_{15/50} and a magnetic flux density B₅₀ by a 25 cm Epstein apparatus, the results of which are also shown in Table 1.

As seen from Table 1, non-oriented electrical steel sheets having excellent magnetic properties can be obtained by controlling a chemical composition of a raw steel material to the ranges of the invention even if the hot band annealing is omitted.

**Table 1**

| Nº | Chemical composition (mass%) | | | | | | | | | | Magnetic properties | | Remarks |
|---|---|---|---|---|---|---|---|---|---|---|---|---|---|
| | C | P | Si | Mn | Al | N | S | Ga | Sn,Sb,Ca,REM,Mg | Ni,Co,Cu,Cr | Iron loss W_{15/50} (W/kg) | Magnetic flux density B₅₀(T) | |
| 1 | 0.0029 | 0.01 | 3.02 | 0.255 | 0.19 | 0.0019 | 0.0019 | 0.0001 | tr. | tr. | 2.75 | 1.701 | Invention Example |
| 2 | 0.0024 | 0.02 | 2.97 | 0.210 | 0.20 | 0.0020 | 0.0018 | 0.0003 | tr. | tr. | 2.96 | 1.673 | Invention Example |
| 3 | 0.0028 | 0.01 | 3.00 | 0.248 | 0.006 | 0.0022 | 0.0022 | 0.0001 | tr. | tr. | 2.79 | 1.706 | Invention Example |
| 4 | 0.0025 | 0.02 | 2.99 | 0.251 | 0.003 | 0.0020 | 0.0023 | 0.0001 | tr. | tr. | 2.72 | 1.718 | Invention Example |
| 5 | 0.0026 | 0.01 | 2.97 | 0.251 | 0.001 | 0.0021 | 0.0021 | 0.0001 | tr. | tr. | 2.64 | 1.731 | Invention Example |
| 6 | 0.0023 | 0.02 | 3.04 | 0.252 | 0.18 | 0.0022 | 0.0019 | 0.0007 | tr. | tr. | 3.23 | 1.651 | Comparative Example |
| 7 | 0.0024 | 0.01 | 3.03 | 0.251 | 0.001 | 0.0017 | 0.0023 | 0.0006 | tr. | tr. | 3.26 | 1.661 | Comparative Example |
| 8 | 0.0023 | 0.01 | 1.52 | 0.256 | 0.24 | 0.0021 | 0.0024 | 0.0001 | tr. | tr. | 3.01 | 1.738 | Invention Example |
| 9 | 0.0025 | 0.02 | 1.49 | 0.252 | 0.007 | 0.0019 | 0.0024 | 0.0001 | tr. | tr. | 3.06 | 1.745 | Invention Example |
| 10 | 0.0025 | 0.01 | 1.45 | 0.254 | 0.001 | 0.0018 | 0.0022 | 0.0001 | tr. | tr. | 2.92 | 1.768 | Invention Example |
| 11 | 0.0025 | 0.01 | 1.54 | 0.247 | 0.22 | 0.0018 | 0.0016 | 0.0006 | tr. | tr. | 3.53 | 1.687 | Comparative Example |
| 12 | 0.0220 | 0.02 | 2.99 | 0.249 | 0.26 | 0.0020 | 0.0019 | 0.0001 | tr. | tr. | 4.04 | 1.651 | Comparative Example |
| 13 | 0.0028 | 0.22 | 2.98 | 0.252 | 0.19 | 0.0023 | 0.0019 | 0.0001 | tr. | tr. | Cannot be rolled due to embrittlement | | Comparative Example |
| 14 | 0.0031 | 0.02 | 3.03 | 3.210 | 0.21 | 0.0021 | 0.0021 | 0.0001 | tr. | tr. | Cannot be rolled due to embrittlement | | Comparative Example |
| 15 | 0.0027 | 0.02 | 3.02 | 0.251 | 2.21 | 0.0023 | 0.0020 | 0.0001 | tr. | tr. | Cannot be rolled due to embrittlement | | Comparative Example |
| 16 | 0.0028 | 0.03 | 2.94 | 0.255 | 0.21 | 0.0054 | 0.0027 | 0.0001 | tr. | tr. | 3.79 | 1.659 | Comparative Example |
| 17 | 0.0022 | 0.03 | 3.05 | 0.252 | 0.19 | 0.0016 | 0.0130 | 0.0001 | tr. | tr. | 3.72 | 1.661 | Comparative Example |
| 18 | 0.0031 | 0.02 | 3.02 | 0.247 | 0.001 | 0.0020 | 0.0021 | 0.0001 | Sn:0.04 | tr. | 2.58 | 1.745 | Invention Example |
| 19 | 0.0035 | 0.01 | 2.97 | 0.256 | 0.001 | 0.0021 | 0.0026 | 0.0001 | Sb:0.03 | tr. | 2.59 | 1.743 | Invention Example |
| 20 | 0.0032 | 0.02 | 3.06 | 0.249 | 0.001 | 0.0022 | 0.0030 | 0.0001 | Sn:0.03, Sb:0.03 | tr. | 2.53 | 1.756 | Invention Example |
| 21 | 0.0027 | 0.01 | 3.02 | 0.255 | 0.001 | 0.0024 | 0.0030 | 0.0001 | Sn:0.04, Ca:0.003 | tr. | 2.52 | 1.753 | Invention Example |
| 22 | 0.0024 | 0.02 | 3.04 | 0.25 | 0.001 | 0.0021 | 0.0025 | 0.0001 | Sn:0.04, REM:0.004 | tr. | 2.52 | 1.755 | Invention Example |
| 23 | 0.0023 | 0.02 | 2.94 | 0.245 | 0.001 | 0.0017 | 0.0022 | 0.0001 | Sn:0.03, Mp:0.005 | tr. | 2.51 | 1.754 | Invention Example |
| 24 | 0.0028 | 0.02 | 2.99 | 0.247 | 0.001 | 0.0019 | 0.0018 | 0.0001 | tr. | Ni:0.03 | 2.55 | 1.729 | Invention Example |
| 25 | 0.0034 | 0.02 | 2.98 | 0.245 | 0.001 | 0.0023 | 0.0018 | 0.0001 | tr. | Ni:1.48 | 2.31 | 1.731 | Invention Example |
| 26 | 0.0030 | 0.01 | 3.03 | 0.251 | 0.001 | 0.0019 | 0.0023 | 0.0001 | tr. | Co:0.03 | 2.56 | 1.730 | Invention Example |
| 27 | 0.0027 | 0.01 | 3.02 | 0.252 | 0.001 | 0.0024 | 0.0021 | 0.0001 | tr. | Co:1.51 | 2.30 | 1.729 | Invention Example |
| 28 | 0.0023 | 0.01 | 3.03 | 0.252 | 0.001 | 0.0025 | 0.0021 | 0.0001 | tr. | Cu:0.05 | 2.53 | 1.730 | Invention Example |
| 29 | 0.0026 | 0.02 | 3.00 | 2.540 | 0.001 | 0.0025 | 0.0022 | 0.0001 | tr. | Cu:1.55 | 2.31 | 1.731 | Invention Example |
| 30 | 0.0026 | 0.02 | 3.04 | 0.250 | 0.001 | 0.0021 | 0.0019 | 0.0001 | tr. | Cr:0.11 | 2.53 | 1.730 | Invention Example |
| 31 | 0.0033 | 0.02 | 2.99 | 0.252 | 0.001 | 0.0021 | 0.0023 | 0.0001 | tr. | Cr:1.52 | 2.29 | 1.730 | Invention Example |

## Claims

1. A non-oriented electrical steel sheet having a chemical composition comprising C: not more than 0.01 mass%, Si: not more than 6 mass%, Mn: 0.05-3 mass%, P: not more than 0.2 mass%, Al: not more than 2 mass%, N: not more than 0.005 mass%, S: not more than 0.01 mass%, Ga: not more than 0.0005 mass%, and optionally one or two of Sn: 0.01-0.2 mass% and Sb: 0.01-0.2 mass%, and optionally one or more selected from Ca: 0.0005-0.03 mass%, REM: 0.0005-0.03 mass% and Mg: 0.0005-0.03 mass%, and optionally one or more selected from Ni: 0.01-2.0 mass%, Co: 0.01-2.0 mass%, Cu: 0.03-5.0 mass% and Cr: 0.05-5.0 mass% in addition to the above chemical composition, and the remainder being Fe and inevitable impurities.

2. The non-oriented electrical steel sheet according to claim 1, wherein Al content is not more than 0.005 mass%.

## Patentansprüche

1. Nicht kornorientiertes Elektroblech mit einer chemischen Zusammensetzung, die umfasst: C: nicht mehr als 0,01 Masse%, Si: nicht mehr als 6 Masse%, Mn: 0,05-3 Masse%, P: nicht mehr als 0,2 Masse%, Al: nicht mehr als 2 Masse%, N: nicht mehr als 0,005 Masse%, S: nicht mehr als 0,01 Masse%, Ga: nicht mehr als 0,0005 Masse% und optional eines oder zwei von Sn: 0,01-0,2 Masse% und Sb: 0,01-0,2 Masse% und optional eines oder mehrere, ausgewählt aus Ca: 0,0005-0,03 Masse%, SEM: 0,0005-0,03 Masse% und Mg: 0,0005-0,03 Masse%, und optional eines oder mehrere, ausgewählt aus Ni: 0,01-2,0 Masse%, Co: 0,01-2,0 Masse%, Cu: 0,03-5,0 Masse% und Cr: 0,05-5,0 Masse%, zusätzlich zu der obenstehenden chemischen Zusammensetzung, wobei der Rest Fe und unvermeidbare Verunreinigungen ist/sind.

2. Nicht kornorientiertes Elektroblech nach Anspruch 1, wobei der Al-Gehalt nicht mehr als 0,005 Masse% beträgt.

## Revendications

1. Tôle d'acier électrique non orientée ayant une composition chimique comprenant : C : pas plus de 0,01 % en masse, Si : pas plus de 6 % en masse, Mn : 0,05 à 3 % en masse, P : pas plus de 0,2 % en masse, Al : pas plus de 2 % en masse, N : pas plus de 0,005 % en masse, S : pas plus de 0,01 % en masse, Ga : pas plus de 0,0005 % en masse, et facultativement un ou deux parmi : Sn : 0,01-0,2 % en masse et Sb : 0,01-0,2 % en masse, et facultativement un ou plusieurs sélectionnés parmi : Ca : 0,0005 à 0,03 % en masse, REM : 0,0005 à 0,03 % en masse et Mg : 0,0005 à 0,03 % en masse, et facultativement un ou plusieurs sélectionnés parmi : Ni : 0,01 à 2,0 % en masse, Co : 0,01 à 2,0 % en masse, Cu : 0,03 à 5,0 % en masse et Cr : 0,05 à 5,0 % en masse, en plus de la composition chimique ci-dessus, et le reste étant du Fe et des impuretés inévitables.

2. Tôle d'acier électrique non orientée selon la revendication 1, dans laquelle la teneur en Al n'est pas supérieure à 0,005 % en masse.
